

## UNITED STATES PATENT OFFICE.

KATHARINA WICKEL, GEB. HOLECEK, OF FEUCHT, NEAR NUEREMBERG, GERMANY.

## MANUFACTURE OF METAL-COATED PAPER.

No Drawing.

Application filed August 5, 1922. Serial No. 572,941.

*To all whom it may concern:*

Be it known that I, KATHARINA WICKEL, geb. HOLECEK, residing at Feucht, near Nuremberg, Bavaria, Germany, have invented certain new and useful Improvements in the Manufacture of Metal-Coated Paper, of which the following is a specification.

The invention relates to an improvement in the manufacture of metal-coated or metallized paper and the like.

The application of metal powders, more particularly bronze, to other materials, for instance paper, in such a manner that they do not lose their original lustre offers great difficulties, as metal powders easily oxidize.

Only very few substances have hitherto shown themselves at all suitable as binders for metal powders and all the known substances show serious drawbacks.

Of the hitherto employed and known binders for this purpose may be mentioned: glue, casein, starch paste, resin, shellac and alcoholic shellac solution.

The metallized paper produced with these binders is, however, permeable and very sensitive to water, the materials themselves are very expensive and the metallized paper soon loses its metallic lustre.

The object of the present invention is a new process in which instead of the hitherto known binding agents for metal powders, like glue, casein, starch, shellac solution and the like, bituminous substances are employed.

The term bitumen is in the first place meant to cover such substances of fossile origin, which are derived from petroleum and which are known under the description of petroleum pitch, the harder pitches of earlier origin of the same series being called asphalt.

The purified product which may be obtained under the trade description "Vulka-bitumen" has shown itself particularly useful. Such bituminous substances are according to this invention either employed in the pure, that means melted state, or dissolved in hydrocarbons, carbon tetrachloride, trichloride ethylene and similar solvents, which do not give off oxygen.

It has been ascertained that such bituminous substances possess physical properties which enable metal-coated papers of an extraordinary large range of utilization to be produced in a very simple and cheap manner.

The improved binder possesses amongst others the extraordinary valuable quality,

which is in itself almost unique, that it does not rob brilliantly shining metal powders of their natural lustre, but even increases it, which is particularly apparent when bituminous substances are employed in conjunction with solvents which do not give off oxygen, as for instance carbon tetrachloride. The metals applied to the paper by means of these binders are permanently protected against oxidation.

A further great advantage is the great binding capacity and the extraordinary great elasticity of the bitumen:

The great viscosity of the dissolved or melted bitumen accounts for an area covering capacity, which far exceeds the known and normal degree, so that for a given surface the expenditure of metal powder and of binding material for the metal coat is very small indeed. As on the other hand and in contradistinction to the hitherto known binders the bituminous substances of the petroleum series possess very different degrees of softness (the melting points lie between 70 and 130° and even higher) metal-coated papers ranging from the pliability of wax paper to the stiffness of card-board may be produced. If the hardest kind of asphalt is employed, the metal may by the subsequent application of friction have an artificial lustre imparted to it. The metal-coated paper prepared according to the new process possesses the property of absolute impermeability to water, oil and air. It has no odour and may therefore be employed for packing food, especially as it can be made very thin and pliable.

This new bitumen metal-coated paper forms the link between the soft wax-paper and the metal-coated paper or the metal foil (tin foil). To the former it is far superior on account of its metallic lustre and the greater resistance against heat and to the ordinary metal-coated paper on account of its softness and flexibility.

It has also been ascertained that by applying high temperatures a firmly fixed bitumen metal-coating may easily and firmly be detached from its paper foundation and be transferred to another article, in such a manner, that the transfer of a design, for instance by heated dies, takes place in clearly defined outlines and that the transferred metal impression retains its natural high lustre and is permanently protected against oxidation. The new metal-coated paper

produced according to the herein described process is therefore a very efficient substitute for genuine leaf-gold, while at the same time it forms a paper for producing metal-  
5 impression, which is far superior to the hitherto known paper for the same object.

By the utilization of the lustre preserving properties of the bitumen and the high melting point a metal impression paper  
10 may easily and cheaply be manufactured from a solution in a single operation.

The prices of the bituminous substances from petroleum tar to asphalt are about one tenth of those for glue and one fortieth  
15 of those for shellac.

In carrying out the invention it may be applied to all hitherto known processes for manufacturing metal-coated paper and the like.

20 So may, for instance, powdered metal (bronze) be stirred into a solution of Vulkabitumen in carbon tetrachloride or the like, and then be applied to paper in any known manner, for instance, by rollers, brushes, scrapers or by compressed air atomizers. Or the metallization may equally well be carried out according to the dry process. The bitumen then takes the place of the hitherto employed resin film and is then  
25 30 further treated in exactly the same manner.

The employment of bitumen offers here also the advantage that a solvent is rendered entirely or partly unnecessary, whereby a considerable saving is effected. Owing to the high viscosity of melted Vulk- or other bitumen or bitumen mixed with very little solvent in the heated state the required film may be directly applied to the paper and the metal powder may then be added by means of suitable apparatus.

35 40 What I claim is:

1. As a new article of manufacture a metal-coated paper whose surface consists of metal powder and a binder of bituminous substance.

2. As a new article of manufacture a polished metal-coated paper whose surface consists of a metal powder and hard asphalt.

3. As a new article of manufacture a transfer paper having a metallic surface consisting of metal powder and bitumen of a high melting point.

In testimony whereof I affix my signature.

FRAU KATHARINA WICKEL, geb. HOLECEK.

Witnesses:

ALEXANDER DE SOTO,  
ALBERT HALSTEAD.